

# UNITED STATES PATENT OFFICE.

JOHN I. CRABTREE, OF ROCHESTER, NEW YORK, ASSIGNOR TO EASTMAN KODAK COMPANY, OF ROCHESTER, NEW YORK, A CORPORATION OF NEW YORK.

## FLASH-POWDER.

1,240,027.

Specification of Letters Patent. Patented Sept. 11, 1917.

No Drawing.

Application filed December 11, 1916. Serial No. 136,384.

To all whom it may concern:

Be it known that I, JOHN I. CRABTREE, a resident of Rochester, in the county of Monroe and State of New York, have invented 5 new and useful Improvements in Flash-Powders, of which the following is a specification.

This invention relates to combustible substances, such as flash powders, that are used 10 to furnish light in photography and other arts. One object of my invention is to provide a flash powder for illuminating purposes which will be an efficient illuminant for various types of photographic work, but 15 will be particularly useful in the art of making photographs in colors, such, for example, as in those color portraiture processes which have been standardized to use nitrogen tungsten incandescent electric lamps. An 20 other object is to provide a safe and convenient packaging of the powder, allowing transportation and handling without danger of premature ignition.

With these and other objects in view, as 25 will hereinafter appear, I have discovered a flash powder the light from which gives practically the same results in spectroscopic tests as the light from nitrogen tungsten lamps, while at the same time the powder 30 possesses all other indispensable characteristics, viz., high actinic value of flash, rapid and reliable speed of combustion, minimum noise, minimum smoke, and practical immunity to premature ignition by friction 35 and percussion. The powder is intended to be used not only in place of nitrogen tungsten lamps, where the latter are not available, or to assist the latter where modified lightings and shorter exposures are desired, but 40 also as an illuminant for photographing with color-sensitive plates and in general wherever an ordinary powder is used.

Flash light illumination is commonly carried out in two ways, (a) by burning metals 45 in free oxygen as in a blow lamp, and (b) by burning metals along with modifying agents when mixed with substances containing combined oxygen, said agents modifying the indispensable characteristics of the 50 powder hereinabove set forth. My powder is of the latter type. In this class of powders mixtures have been proposed of many different combustible metals with various kinds of oxidizing and modifying agents, 55 but extensive testing of these proposed mix-

tures has shown that they are deficient in certain respects. Either they do not furnish sufficient red light rays, or they lack some of the other essentials, producing, for instance, excessive smoke or a loud explosion, or costing too much for raw materials. My invention is intended to obviate these disadvantages and to provide a flash powder composition possessing all the properties that are considered necessary for photographic purposes. 60 65

One illustrative embodiment of this invention includes the following ingredients, which may be mixed in the proportions indicated as parts by weight:

|                                  |     |       |
|----------------------------------|-----|-------|
| Sodium oxalate                   | 4   | parts |
| Red phosphorus                   | 3.5 | "     |
| Magnesium                        | 5   | "     |
| Aluminum                         | 10  | "     |
| Strontium nitrate (crys-<br>tal) | 40  | "     |

It is best that the ingredients be dry, free from lumps, and powdered to pass through a fine sieve. Furthermore, the red phosphorus should have been freed from yellow phosphorus, as by washing with caustic alkali. For homogeneity, the ingredients should preferably be mixed in the order given in the formula, the oxalate and red 80 phosphorus being first stirred together, then the metals added, and finally the strontium nitrate shaken in.

While I have described the preferred embodiment of my invention, many variations 90 falling within the scope of the appended claims will occur to those skilled in this art. For example, the red light in the flash may be slightly adjusted by varying the sodium oxalate or by partial substitution of the 95 strontium nitrate, or other oxygen yielding salt of strontium, by barium nitrate. Where speed or comparative freedom from smoke is not particularly needed, the phosphorus may be wholly or partly replaced by red 100 antimony sulfid or the sodium oxalate may be wholly or partly replaced by sodium benzoate, naphthalene, or sodium tungstate. The sodium oxalate, or one of its equivalents, has been found necessary, to make the 105 light from the flash give, for practical purposes, the same spectroscopic results as the light from nitrogen tungsten lamps. It also adds to the ease or smoothness of burning of the powder and accomplishes these re- 110

sults without impairing the other characteristic essential to a commercial flash powder. It may be noted that phosphorus and antimony sulfid are examples of easy 5 burning substances which facilitate ignition and complete combustion.

In cases where speed is not required, as, for instance, still life subjects, a modification of my invention may be:

|    |                   |     |       |
|----|-------------------|-----|-------|
| 10 | Sodium oxalate    | 5   | parts |
|    | Red phosphorus    | 2.5 | "     |
|    | Aluminum          | 15  | "     |
|    | Strontium nitrate | 40  | "     |

15 This mixture is relatively slow but highly actinic and possesses the desired spectrum. From the above formulæ it is evident that aluminum and mixtures of aluminum with magnesium act equivalently in these powders, so far as spectroscopic results are concerned, the essential fact being that a combustible metal of high actinic value is mixed 20 with my oxidizing and modifying agents.

If the powder is made up to be kept for 25 future use or to be transported, the strontium nitrate of one charge should be inclosed in one package or compartment and the mixture of the other ingredients of that charge inclosed in a separate package or 30 compartment. The contents of these two complementary packages are shaken together just prior to use. Putting up the powders in this way in two parts renders them immune to premature ignition by friction or percussion.

The powder may be used in any customary 35 way, being laid, for example, in piles or trains, in open apparatus or in flash bags or flash cabinets, and preferably ignited 40 electrically or by flame. Ten grams of the powder ignited in a flash bag have been found sufficient, owing to its high actinic qualities, for taking a color portrait with a lens aperture of f. 6, though, of course, 45 the amount will vary somewhat with other factors.

If powder of the characteristics set forth in the first formula above given is used, the effective duration of the flash averages about 50 1/20 of a second, a speed which is sufficient

to avoid defective photographs due to blinking and movement of nervous subjects in portraiture. Even when burned in relatively large lots, it has been found to be practically silent with but a small amount 55 of smoke. Tests in a color camera and with a wedge spectrograph show that spectrographically the light from the flash is almost an exact duplicate of light from the nitrogen tungsten lamp.

60 The speed of the oxidation or chemical reaction, which takes place when the powder is burned, determines the duration of the flash and can be varied by changing the relative proportions of magnesium and 65 aluminum, or by altering the degree of fineness of the metals, or by both varying the proportions and fineness of the metals. For example, the greater the proportion of magnesium or the finer its state of subdivision 70 the shorter will be the duration of the flash. Hence, a very useful and exact adjustment of the speed of my powder to the requirements imposed by the particular circumstances, under which it is to be used, may 75 be easily made.

I claim:

1. A flash powder comprising combustible metal of high actinic value, phosphorus, an alkali earth metal nitrate, and a sodium 80 salt, the effect of which on the flash is substantially like that of sodium oxalate.

2. A flash powder mixture of sodium oxalate, phosphorus, combustible metal of high actinic value, and an alkali-earth metal nitrate.

3. A flash powder mixture of sodium oxalate, phosphorus, combustible metal of high actinic value, and strontium nitrate.

4. A flash powder comprising sodium oxalate, red phosphorus, magnesium, aluminum and strontium nitrate.

5. A flash powder composed substantially of strontium nitrate 40 parts, sodium oxalate 4 parts, red phosphorus 3.5 parts, magnesium 5 parts and aluminum 10 parts.

JOHN I. CRABTREE.

Witnesses:

G. C. COOKE,  
R. L. STINCHFIELD.